

# UNITED STATES PATENT OFFICE.

WALTER GLAESER, OF BROOKLYN, NEW YORK.

## FLEXIBLE TRANSPARENT MATERIAL AND METHOD OF MAKING SAME.

1,303,053.

Specification of Letters Patent.

Patented May 6, 1919.

No Drawing.

Application filed September 19, 1917. Serial No. 192,181.

To all whom it may concern:

Be it known that I, WALTER GLAESER, a subject of the German Emperor, and a resident of Brooklyn, county of Kings, and State of New York, have invented a new and useful Improvement in Flexible Transparent Material and Methods of Making Same, of which the following is a specification, the principle of the invention being herein explained and the best mode in which I have contemplated applying that principle, so as to distinguish it from other inventions.

The present invention, relating as indicated to a flexible transparent material and method of making same is concerned more particularly with such a material, which is adapted to constitute a screen for motion-pictures, although, obviously, its use is in no way limited to that field and other uses and adaptations of it will readily suggest themselves to those skilled in the various arts. To the accomplishment of the foregoing and related ends, said invention, then, consists of the means hereinafter fully described and particularly pointed out in the claim.

The following description sets forth in detail one approved method of carrying out the invention, such disclosed method, however, constituting but one of various ways in which the principle of the invention may be used.

To make my improved material I take one part of glue, which may be either bleached or unbleached, and let the same soak in about one and one-half parts of water for at least twenty-four hours. At the end of this time another one and one-half parts of water are added and the mixture is heated by indirect heat, as in a double boiler, until a clear solution is obtained. To this solution I add from a quarter to one whole part of glycerin, and it is desirable that the glycerin be vigorously stirred into the mixture. The amount of glycerin which should be added is determined by the elasticity which is desired in the final product, and the greater amount of glycerin used, the higher the elasticity of the finished material. This mixture of glue, water and glycerin is now heated again over an indirect fire until its bulk amounts to about two and one-half parts when the mixture is allowed to cool until it begins to form a relatively thin jelly.

In a separate container one-half part of strong formaldehyde is mixed with an equal amount of water and this mixture is then stirred quickly into the cold glue and glycerin mixture, and the resulting material is spread on a cold glass plate to any desired thickness. It is desirable that the spreading operation be performed as rapidly as possible as otherwise the mixture may harden before it can be properly spread and smoothed.

If the screen to be made is of very great size it is desirable to reinforce the mixture on the glass plate by placing a sheet of unglued paper, bolting silk or similar material on the film on the plate, and this material is then covered by a second layer of the mixture.

After the solution has been applied to the plate it should be kept in air that is free from dust for a short time, about fifteen minutes or so, until the material has become somewhat hard, when the plate and coating are placed in a drying closet and dried at about 200 degrees F. Under this drying temperature the material hardens and materially toughens and forms a very effective screen.

Other forms may be employed embodying the features of my invention instead of the one here explained, change being made in the form or construction, provided the elements stated by the following claim or the equivalent of such stated elements be employed, whether produced by my preferred method or by others embodying steps equivalent to those stated in the following claim.

I therefore particularly point out and distinctly claim as my invention:

In a method of making a flexible transparent material, the steps which consist in soaking one part of glue in one and one half parts of water, adding another one and one half parts of water and heating the mixture indirectly until a clear solution is formed, stirring into the solution one fourth part or more of glycerin, heating such mixture to a bulk of two and one half parts, cooling the same and adding formaldehyde.

Signed by me, this 13th day of September, 1917.

WALTER GLAESER.